

## 1

3,227,531

### MOTOR FUEL COMPOSITION

Louis N. Calvino, Plainfield, and John D. Turner, North Plainfield, N.J., assignors to Esso Research and Engineering Company, a corporation of Delaware  
No Drawing. Filed July 18, 1961, Ser. No. 124,816  
4 Claims. (Cl. 44—58)

The present invention relates to improved motor fuels and a method of operating an engine which tends to promote engine cleanliness and particularly to gasoline compositions for internal combustion engines containing improved solvent oils of enhanced stability. More particularly, the instant invention concerns improved hydrocarbon solvent oils having incorporated therein stabilizing amounts of a polymeric additive.

Solvent oils, both synthetic and hydrocarbonaceous, are commonly employed in minor amounts as motor and aviation fuel additives to serve as a general purpose, upper cylinder lubricant to reduce valve stem and piston ring sticking and to decrease manifold and intake port deposits. One of the primary functions of these motor fuel solvent oils is to aid by selective solvent action in the removal of gum, resins, varnishes and sludge. However, oxygenated gums and resins are not readily removed by these solvent oils, and it would be highly desirable to employ as a solvent oil, or as an adjuvant to solvent oils, a stable composition that has high specificity for gums and varnishes. In the past, various oxygenated solvents have been added to gasoline for this purpose, but these materials have not been wholly effective, either because of too high vapor pressure at motor operating conditions, or because excessive quantities were required. Thus, it has been suggested that high boiling esters such as amyl stearate be employed as a solvent oil. Such esters, however, have not given satisfaction and their solvent powers are inadequate.

The need for a highly active stable solvent oil type additive has been long recognized. A tendency to cause manifold deposit and intake port deposit buildup represents a serious fuel deficiency, particularly when the fuel is used in low temperature service with considerable engine idling time. Catalytically cracked gasolines which have comparatively high octane numbers and are thus widely used are unstable and require the use of an antioxidant. Both these unstable fuels and antioxidant residues contribute to manifold deposits. Use of a solvent oil type additive represents a desirable method of minimizing these deposits.

It has now been discovered that superior solvent oils may be prepared by incorporating minor amounts of a high molecular weight, ashless, oil soluble polymeric additive in the solvent oil. In particular, it has been found that those high molecular weight, ashless, oil soluble polymers which function as multifunctional viscosity index improvers in heavy lubricating oils are surprisingly effective in promoting overall intake and fuel system cleanliness and in enhancing the oxidation stability of solvent oils. More particularly, it has been found that the addition of small quantities to a light mineral distillate solvent oil or upper cylinder lubricant of a terpolymer of maleic anhydride, vinyl ester and alkyl fumarate enhances the stability characteristics of the solvent oil and the motor fuel in which the solvent oil is employed.

This is a significant and surprising discovery, since

## 2

the use of high molecular weight polymeric materials in light solvent oils and volatile fuels has been avoided in the past in the belief that such additives would increase the amount of combustion and manifold deposits and promote the formation of additional sludge and deposits. Additionally, it was believed that polymeric type additives would fail to function as detergents or dispersants in a volatile fuel like gasoline, especially after being combusted at high temperatures in a combustion chamber.

10 The advantages of the present invention allow an improved solvent oil to be added to gasoline fuels, and the polymeric additive to have multifunctional properties in stabilizing the solvent oil against excessive oxidation, 15 reducing manifold or intake system deposits, and additionally promoting overall fuel system and carburetor cleanliness and also throughout those engine areas not having direct liquid contact with the heavy crankcase lube oil. The present invention also allows for reduced 20 quantities of the polymeric additives to be employed in a more effective direct manner in reducing sludge and sediment. Previous to this discovery, polymeric additives in general were restricted to heavy lubricating oils to aid in suspending the sludge derived from the original 25 volatile fuel composition, such as the unstable cracked fuel components, the additive in the fuel such as the antioxidant, and the combustion and blow-by products of the fuel. The applicants have thus discovered a direct method of both promoting fuel system, intake system and engine cleanliness and enhancing solvent oil 30 stability.

35 The solvent oils in which the polymeric additive of the instant invention may be beneficially employed comprise synthetic and mineral solvent oils having an SUS viscosity of between about 50 and 2000 at 100° F., e.g. 50 to 500, and those having an SUS viscosity of about 30 to 150 at 210° F., and a Conradson carbon content of less than 1 wt. percent. The synthetic solvent oils include those oxygenated nonvolatile compounds such as 40 fatty acid esters like amyl stearate; ester type oxidates derived from deoiled macrocrystalline wax as set forth in U.S. Patent 2,965,458; polyoxyalkylene compounds as in U.S. Patents 2,807,525 and 2,807,526; and other 45 organic, oil soluble, oxygenated, high solvency types of nonvolatile compounds and mixtures thereof.

These synthetic solvent oils also include those liquid synthesis products derived from the Oxo processes as set forth in U.S. Patent 2,955,928 and those Oxo bottoms acylated by treatment with ketene or acetic anhydride and the like as set forth in U.S. application Serial No. 15,527, filed March 17, 1960, now U.S. Patent No. 3,054,666. Those high molecular weight esters, ethers, alcohols, aldehydes, preferably saturated having more than an average of 16 carbon atoms per molecule 50 and boiling above about 250° F. are the preferred synthetic solvent oils.

55 The petroleum solvent oils may be a naphthene base distillate, a paraffin base distillate or mixtures thereof. These solvent oils are completely obtained by vacuum distillation of the base oil at from 20 to 40 mm. pressure and subsequent acid treatment, caustic washing or hydrofining or any combination of the distillate. These mineral oils may also comprise those silica gel extracted 60 bright stocks obtained by the select silica gel treatment of a deasphalted, solvent extracted, dewaxed virgin residual or bright stock as described in U.S. Patent 65

2,904,493, for example, a bright stock having an SUS viscosity of 1858 at 100° F. and 132 at 210° F.

The preferred solvent oils are those light liquid hydrocarbon mineral distillate oils having an SUS viscosity at 100° F. of between 50 and 300, e.g. 70 to 90. Suitable solvent oils include those oils having a 50% distillation point above 350° F. at 10 mm. Hg pressure, having a Saybolt viscosity at 100° F. not above 450 seconds, and having an API gravity of about 18 to 28°. A typical solvent oil, for example, has the following inspection:

50% distillation point @ 10 mm. Hg, ° F. ----- 413  
Saybolt viscosity @ 100° F., SUS ----- 75.3  
° API gravity ----- 26.6

15 Mineral solvent oils are usually light solvent lubricating oils or low viscosity naphthenic distillates, but may be petroleum, animal or vegetable sources or mixtures thereof. In general, mineral solvent oils have aniline points of 160° F. to 170° F. and API gravities of 25 to 28. Conventional solvent oils are described in U.S. Patent 2,066,234 issued to Sloane and Wasson on December 29, 1936, and U.S. Patents 2,579,692, 2,646,348, and 2,654,697 and others recited which are incorporated by reference.

The solvent oils of the invention may be mineral or synthetic solvent oils as described or combinations thereof such as from 40 to 80% mineral oil or even 50 to 90% mineral oil, and may contain other additives such as detergents; halogenated aromatic compounds; acid tars; oiliness additives; metal deactivators such as N,N'-disalicylidene-1,2-diaminopropane; preignition additives such as alkyl-aryl phosphates like tricresyl phosphate, tri-β-chloroethyl phosphate, amine phosphates, and the like; antioxidants such as 2,6-ditertiary-butyl-4-methyl phenol, N,N'-di-secondary-butyl-para-phenylene diamine, N-butyl para amino phenol, and the like; dyes; antifrust additives such as amines and phosphates and the like; anti-icing agents such as hexylene glycol, isopropanol; antiknocks; and the like.

20 The polymeric additives of this invention are multifunctional V.I. improper additive polymers such as those high molecular weight, ashless, oil soluble polymers obtained by copolymerizing maleic anhydride with an aliphatic ester of an  $\alpha,\beta$ -unsaturated dicarboxylic acid and a copolymerizable C<sub>2</sub> to C<sub>4</sub> alkylene ester of a C<sub>1</sub> to C<sub>6</sub> monocarboxylic acid. The preferred embodiment of this polymer includes the terpolymer obtained by copolymerizing maleic anhydride, vinyl acetate, and C<sub>8</sub> to C<sub>20</sub> alkyl fumarate. The preferred polymeric additive agents are those terpolymers obtained by copolymerizing maleic anhydride, a vinyl ester of a short chain fatty acid, and a long straight chain C<sub>8</sub> to C<sub>20</sub> fatty alcohol ester of a butenedioic acid.

25 It is preferred that the esters of di- and monocarboxylic acids used to form the copolymers of the present invention are so chosen that a mixture of relatively long and short aliphatic side chains is disposed along the polymer chain. The relatively long side chains may be provided by C<sub>8</sub> to C<sub>20</sub> aliphatic saturated or unsaturated, substituted or unsubstituted ester of C<sub>4</sub> to C<sub>6</sub>  $\alpha,\beta$ -unsaturated dicarboxylic acids, e.g. esters derived from C<sub>8</sub> to C<sub>20</sub> fatty alcohols, preferably alkyl alcohols. Straight chain alcohols, branched chain alcohols, or a mixture of the two can be used. The preferred acids are  $\alpha,\beta$ -unsaturated conjugated dicarboxylic acids, such as butenedioic acid like fumaric acid although maleic or itaconic acid may be used. Suitable esters include mono- and di-C<sub>8</sub> Oxo fumarate, tallow fumarate, lauryl maleate, stearyl fumarate, C<sub>13</sub> Oxo fumarate, and cetyl itaconate, and the like. The relatively short side chains are preferably provided by using C<sub>2</sub> to C<sub>6</sub> alkylene esters or ethers of C<sub>1</sub> to C<sub>6</sub> carboxylic acids, preferably vinyl or allyl esters such as allyl and vinyl esters of short chain C<sub>2</sub> to C<sub>4</sub> fatty acids like vinyl acetate and allyl acetate. Minor amounts, e.g. 1 to 10 molar proportions of other ethyl-

30 4  
5  
6  
7  
8  
9  
10  
11  
12  
13  
14  
15  
16  
17  
18  
19  
20  
21  
22  
23  
24  
25  
26  
27  
28  
29  
30  
31  
32  
33  
34  
35  
36  
37  
38  
39  
40  
41  
42  
43  
44  
45  
46  
47  
48  
49  
50  
51  
52  
53  
54  
55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
698  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
779  
779  
780  
781  
782  
783  
784  
785  
786  
787  
788  
789  
789  
790  
791  
792  
793  
794  
795  
796  
797  
798  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
879  
879  
880  
881  
882  
883  
884  
885  
886  
887  
888  
889  
889  
890  
891  
892  
893  
894  
895  
896  
897  
898  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
979  
979  
980  
981  
982  
983  
984  
985  
986  
987  
988  
989  
989  
990  
991  
992  
993  
994  
995  
996  
997  
998  
999  
1000  
1001  
1002  
1003  
1004  
1005  
1006  
1007  
1008  
1009  
1009  
1010  
1011  
1012  
1013  
1014  
1015  
1016  
1017  
1018  
1019  
1019  
1020  
1021  
1022  
1023  
1024  
1025  
1026  
1027  
1028  
1029  
1029  
1030  
1031  
1032  
1033  
1034  
1035  
1036  
1037  
1038  
1039  
1039  
1040  
1041  
1042  
1043  
1044  
1045  
1046  
1047  
1048  
1049  
1049  
1050  
1051  
1052  
1053  
1054  
1055  
1056  
1057  
1058  
1059  
1059  
1060  
1061  
1062  
1063  
1064  
1065  
1066  
1067  
1068  
1069  
1069  
1070  
1071  
1072  
1073  
1074  
1075  
1076  
1077  
1078  
1079  
1079  
1080  
1081  
1082  
1083  
1084  
1085  
1086  
1087  
1088  
1089  
1089  
1090  
1091  
1092  
1093  
1094  
1095  
1096  
1097  
1098  
1099  
1100  
1101  
1102  
1103  
1104  
1105  
1106  
1107  
1108  
1109  
1109  
1110  
1111  
1112  
1113  
1114  
1115  
1116  
1117  
1118  
1119  
1119  
1120  
1121  
1122  
1123  
1124  
1125  
1126  
1127  
1128  
1129  
1129  
1130  
1131  
1132  
1133  
1134  
1135  
1136  
1137  
1138  
1139  
1139  
1140  
1141  
1142  
1143  
1144  
1145  
1146  
1147  
1148  
1149  
1149  
1150  
1151  
1152  
1153  
1154  
1155  
1156  
1157  
1158  
1159  
1159  
1160  
1161  
1162  
1163  
1164  
1165  
1166  
1167  
1168  
1169  
1169  
1170  
1171  
1172  
1173  
1174  
1175  
1176  
1177  
1178  
1179  
1179  
1180  
1181  
1182  
1183  
1184  
1185  
1186  
1187  
1188  
1189  
1189  
1190  
1191  
1192  
1193  
1194  
1195  
1196  
1197  
1198  
1199  
1200  
1201  
1202  
1203  
1204  
1205  
1206  
1207  
1208  
1209  
1209  
1210  
1211  
1212  
1213  
1214  
1215  
1216  
1217  
1218  
1219  
1219  
1220  
1221  
1222  
1223  
1224  
1225  
1226  
1227  
1228  
1229  
1229  
1230  
1231  
1232  
1233  
1234  
1235  
1236  
1237  
1238  
1239  
1239  
1240  
1241  
1242  
1243  
1244  
1245  
1246  
1247  
1248  
1249  
1249  
1250  
1251  
1252  
1253  
1254  
1255  
1256  
1257  
1258  
1259  
1259  
1260  
1261  
1262  
1263  
1264  
1265  
1266  
1267  
1268  
1269  
1269  
1270  
1271  
1272  
1273  
1274  
1275  
1276  
1277  
1278  
1279  
1279  
1280  
1281  
1282  
1283  
1284  
1285  
1286  
1287  
1288  
1289  
1289  
1290  
1291  
1292  
1293  
1294  
1295  
1296  
1297  
1298  
1299  
1300  
1301  
1302  
1303  
1304  
1305  
1306  
1307  
1308  
1309  
1309  
1310  
1311  
1312  
1313  
1314  
1315  
1316  
1317  
1318  
1319  
1319  
1320  
1321  
1322  
1323  
1324  
1325  
1326  
1327  
1328  
1329  
1329  
1330  
1331  
1332  
1333  
1334  
1335  
1336  
1337  
1338  
1339  
1339  
1340  
1341  
1342  
1343  
1344  
1345  
1346  
1347  
1348  
1349  
1349  
1350  
1351  
1352  
1353  
1354  
1355  
1356  
1357  
1358  
1359  
1359  
1360  
1361  
1362  
1363  
1364  
1365  
1366  
1367  
1368  
1369  
1369  
1370  
1371  
1372  
1373  
1374  
1375  
1376  
1377  
1378  
1379  
1379  
1380  
1381  
1382  
1383  
1384  
1385  
1386  
1387  
1388  
1389  
1389  
1390  
1391  
1392  
1393  
1394  
1395  
1396  
1397  
1398  
1399  
1400  
1401  
1402  
1403  
1404  
1405  
1406  
1407  
1408  
1409  
1409  
1410  
1411  
1412  
1413  
1414  
1415  
1416  
1417  
1418  
1419  
1419  
1420  
1421  
1422  
1423  
1424  
1425  
1426  
1427  
1428  
1429  
1429  
1430  
1431  
1432  
1433  
1434  
1435  
1436  
1437  
1438  
1439  
1439  
1440  
1441  
1442  
1443  
1444  
1445  
1446  
1447  
1448  
1449  
1449  
1450  
1451  
1452  
1453  
1454  
1455  
1456  
1457  
1458  
1459  
1459  
1460  
1461  
1462  
1463  
1464  
1465  
1466  
1467  
1468  
1469  
1469  
1470  
1471  
1472  
1473  
1474  
1475  
1476  
1477  
1478  
1479  
1479  
1480  
1481  
1482  
1483  
1484  
1485  
1486  
1487  
1488  
1489  
1489  
1490  
1491  
1492  
1493  
1494  
1495  
1496  
1497  
1498  
1499  
1500  
1501  
1502  
1503  
1504  
1505  
1506  
1507  
1508  
1509  
1509  
1510  
1511  
1512  
1513  
1514  
1515  
1516  
1517  
1518  
1519  
1519  
1520  
1521  
1522  
1523  
1524  
1525  
1526  
1527  
1528  
1529  
1529  
1530  
1531  
1532  
1533  
1534  
1535  
1536  
1537  
1538  
1539  
1539  
1540  
1541  
1542  
1543  
1544  
1545  
1546  
1547  
1548  
1549  
1549  
1550  
1551  
1552  
1553  
1554  
1555  
1556  
1557  
1558  
1559  
1559  
1560  
1561  
1562  
1563  
1564  
1565  
1566  
1567  
1568  
1569  
1569  
1570  
1571  
1572  
1573  
1574  
1575  
1576  
1577  
1578  
1579  
1579  
1580  
1581  
1582  
1583  
1584  
1585  
1586  
1587  
1588  
1589  
1589  
1590  
1591  
1592  
1593  
1594  
1595  
1596  
1597  
1598  
1599  
1600  
1601  
1602  
1603  
1604  
1605  
1606  
1607  
1608  
1609  
1609  
1610  
1611  
1612  
1613  
1614  
1615  
1616  
1617  
1618  
1619  
1619  
1620  
1621  
1622  
1623  
1624  
1625  
1626  
1627  
1628  
1629  
1629  
1630  
1631  
1632  
1633  
1634  
1635  
1636  
1637  
1638  
1639  
1639  
1640  
1641  
1642  
1643  
1644  
1645  
1646  
1647  
1648  
1649  
1649  
1650  
1651  
1652  
1653  
1654  
1655  
1656  
1657  
1658  
1659  
1659  
1660  
1661  
1662  
1663  
1664  
1665  
1666  
1667  
1668  
1669  
1669  
1670  
1671  
1672  
1673  
1674  
1675  
1676  
1677  
1678  
1679  
1679  
1680  
1681  
1682  
1683  
1684  
1685  
1686  
1687  
1688  
1689  
1689  
1690  
1691  
1692  
1693  
1694  
1695  
1696  
1697  
1698  
1699  
1700  
1701  
1702  
1703  
1704  
1705  
1706  
1707  
1708  
1709  
1709  
1710  
1711  
1712  
1713  
1714  
1715<br

described in British Patent 807,737, which is hereby incorporated by reference.

The polymeric additives of this invention are incorporated in minor amounts between 0.1 and 20% by weight in the solvent oil or preferably between 0.5 and 15% by weight, for example, between 2 and 8 wt. percent. The improved solvent oil concentration may vary dependent upon the characteristics of the gasoline, the engine, and the type of driving conditions under which used, but is generally sufficient to reduce or control intake system deposits to an acceptable level. Solvent oils are commonly employed at a concentration of between 0.05 and 3.0 wt. percent and especially between 0.1 and 1.0 wt. percent based on the gasoline blend. The concentration level of the polymeric additive based on the motor fuel ranges between 0.001 and 0.5 wt. percent, and preferred is 0.005 to 0.2 wt. percent.

In carrying out the invention, a small amount of the improved polymeric containing solvent oil is either added directly to the motor or aviation gasoline itself or is injected into the intake system or manifold in any desired manner in order to contact the deposits and gum on the surface. The improved solvent oil of the present invention is also of beneficial use for fluxing gummy deposits and the like from the fuel systems of diesel engines, oil burner installations, jet engines, turbines, and other deposit laden surfaces and, thus, may also be incorporated in diesel fuels, jet fuels, heating oils, and other hydrocarbon oils and fuels. It is, of course, recognized that the polymeric additive may be separately incorporated in the gasoline or in an oil concentrate containing other additives.

The motor fuels in which the polymeric additives are employed in order to reduce the formation of deposits, sludge and varnish are conventional petroleum distillate fuels boiling in the gasoline boiling point range employed in internal combustion, preferably spark ignition, engines. They are supplied in a number of different grades depending upon the type of service for which they are intended. The copolymers may be employed in all of these grades but are particularly useful in motor and aviation gasolines. Motor gasolines as referred to in connection with the present invention are defined by ASTM Specification D-439-58T in Types A, B and C. They are composed of a mixture of various types of hydrocarbons including aromatics, olefins, paraffins, isoparaffins, naphthenes and, occasionally, diolefins. Those motor fuels containing at least 10% by weight of thermally or catalytically high aromatic components may be especially benefited from the instant invention. Suitable gasolines to which the polymeric additives of the instant invention may be added are those gasolines having an octane number range of 83 to 105 or higher, such as a clear octane number of over 90, for example, over 95 or 100, and comprising over 20% by volume of aromatic hydrocarbons and less than 30% by volume of olefinic hydrocarbons. They are derived from petroleum crude oil by refining processes such as fractional distillation, catalytic cracking, hydroforming, alkylation, isomerization, polymerization and solvent extraction. Motor gasolines normally have boiling ranges between about 70° F. and about 450° F., while aviation gasolines have narrower boiling ranges of between 100° and 330° F. The vapor pressures of gasoline as determined by ASTM Method D-86 vary between about 7 and about 15 p.s.i. at 100° F. The copolymers may also be employed in aviation gasoline, which have properties similar to those of motor gasolines but normally have somewhat higher octane numbers and narrower boiling ranges. The properties of aviation gasolines are set forth in U.S. Military Specification MIL-F-5572 and ASTM Specification D-910-57T.

The copolymeric additives employed in accordance with the invention may be used in gasolines with other additive agents conventionally used in such fuels. It is common practice to employ from about 0.5 to about

7.0 cc./gal. of alkyl lead antiknock agents, such as tetraethyl lead, tetramethyl lead, dimethyl diethyl lead or a similar alkyl lead antiknock agent or olefinic lead antiknock agents such as tetravinyl lead, triethyl vinyl lead, and the like, or a combination thereof, in both motor 5 and aviation gasolines, e.g. 1.0 to 3.0 cc. of tetraethyl lead-tetramethyl lead combination. Antiknock agents may also include other organometallic additives containing lead, iron, nickel, lithium, manganese and the like. Other additives such as those conventionally employed in gasolines may be used such as corrosion inhibitors, antioxidants, antistatic agents, lead octane appreciators like t-butyl acetate, auxiliary scavengers like tri- $\beta$ -chloroethyl phosphate, dyes, anti-icing agents like isopropanol, hexylene glycol and the like.

10 Catalytically and thermally cracked and reformed gasolines containing a high aromatic content, whether leaded or unleaded, are particularly prone to yield excessive manifold deposits and are improved by addition of the applicants' solvent oil composition.

15 Lead antiknock agents are usually employed in conjunction with halogenated hydrocarbon scavenger agents boiling in the range between 50 and 250° F., such as ethylene bromide, ethylene chloride, and the like in concentrations of from 0.5 to 3.0 theories, with preferred 20 concentration levels of from 0.8 to 1.5 theories of ethylene bromide used alone or 0.8 to 1.5 of ethylene dichloride and 0.3 to 0.8 of ethylene dibromide when a mixed 25 scavenger is used.

25 The preparation of the high molecular weight polymers may be illustrated by the following examples.

#### EXAMPLE 1

The following monomer mixture is prepared:

|                                    | Percent by wt. |
|------------------------------------|----------------|
| 35 Lauryl fumarate                 | 75.2           |
| Lauryl alcohol (reaction modifier) | 2              |
| Vinyl acetate                      | 18.8           |
| Maleic anhydride                   | 4              |

40 The monomer mixture is then divided into two parts, part A being copolymerized at 60° C. using 1 wt. percent benzoyl peroxide and part B being copolymerized at 90° C. using 0.4 wt. percent tertiary butyl perbenzoate. Copolymerization is continued in both instances until a 45 reaction mixture having a viscosity of 400 stokes at the reaction temperature, and the copolymeric products diluted with an SAE 10 type mineral oil or a solvent oil. The solution is then stripped under a reduced pressure of 5 mm. Hg at 100° C. until the solution contained 50% 50 of the active polymer. The benzoyl peroxide polymer is designated as polymer A with the t-butyl perbenzoate designated as polymer B, each polymer having a chain length of about 3,000 to 10,000 carbon atoms.

#### EXAMPLE 2

The procedure of Example 1 is repeated exactly except that the materials polymerized are as follows:

|                                   | Mole percent |
|-----------------------------------|--------------|
| 60 Di-C <sub>8</sub> Oxo fumarate | 17.8         |
| Di-tallow fumarate                | 7.4          |
| Vinyl acetate                     | 71.8         |
| Maleic anhydride                  | 3.0          |

65 The di-tallow fumarate is prepared by esterifying fumaric acid with alcohols derived from the hydrogenation of tallow. These tallow acids contain a straight chain alcohol mixture comprising about 1 wt. percent C<sub>12</sub> alcohol, 6 wt. percent C<sub>14</sub> alcohol, 30 wt. percent C<sub>16</sub> alcohol, 60 wt. percent C<sub>18</sub> alcohol, and 3 wt. percent C<sub>20</sub> alcohol and had an average molecular weight of about 265. The di-C<sub>8</sub> Oxo fumarate is obtained by esterifying fumaric acid with C<sub>8</sub> Oxo alcohols. The Oxo process for preparing alcohols is described in U.S. Patents 7,232,066, 2,504,682, etc. In brief, the C<sub>8</sub> Oxo alcohols

are prepared by reacting an olefin prepared by the reaction of butylene and propylene with carbon monoxide and oxygen to form a mixture of aldehydes which were hydrogenated. The di-C<sub>8</sub> Oxo fumarate and di-tallow fumarates are mixed. The resulting mixture has an average molecular weight of about 420. Two wt. percent of benzoyl peroxide based on the total weight of the polymerizable materials is used as a catalyst. Two wt. percent of lauryl alcohol based on the total weight of the polymerizable materials is used as a moderator. The polymer was designated as polymer C and has a chain length of 3,000 to 10,000 carbon atoms.

#### EXAMPLE 3

The procedure of Example 2 is repeated exactly except that the materials polymerized are as follows:

|                                 | Mole percent |
|---------------------------------|--------------|
| Di-C <sub>8</sub> Oxo fumarate  | 14.6         |
| Di-C <sub>13</sub> Oxo fumarate | 6.6          |
| Di-tallow fumarate              | 4.0          |
| Vinyl acetate                   | 71.9         |
| Maleic anhydride                | 2.9          |

The di-C<sub>13</sub> Oxo fumarate is prepared by esterifying fumaric acid with a C<sub>13</sub> Oxo alcohol. The C<sub>13</sub> Oxo alcohols are prepared by the Oxo process by reacting propylene tetramer with carbon monoxide and hydrogen to form a branched C<sub>13</sub> aldehyde which is hydrogenated to form the C<sub>13</sub> alcohol. The three fumarates are mixed to obtain a fumarate mixture having an average molecular weight of about 420. This polymer is designated polymer D.

#### EXAMPLE 4

The Sligh test is an accelerated oxidation test which measures the resistance of an oil to oxidation and the formation of sludge. A sample of the oil is placed in a specially constructed vessel which is charged with oxygen. The vessel is then heated in a bath for a specified time and at a specified temperature. At the end the oil is diluted with a light naphtha, filtered and the weight of precipitate reported as the Sligh number in milligrams of precipitate. The effect upon the Sligh number of various gasoline solvent mineral oils with and without the polymeric additives is shown in the following Table I.

Table I

OXIDATION STABILITY OF SOLVENT OILS CONTAINING POLYMERIC ADDITIVES

Sligh No.

|                                            |      |
|--------------------------------------------|------|
| Solvent oil Y <sup>1</sup>                 | 14.3 |
| Solvent oil Y plus 6 wt. percent polymer D | 1.0  |
| Solvent oil X <sup>2</sup>                 | 84.1 |
| Solvent oil X plus 6 wt. percent polymer D | 17.8 |

<sup>1</sup> Solvent oil Y was a coastal distillate of about 80 SUS at 100° F.

<sup>2</sup> Solvent oil X was a methyl ethyl ketone dewaxed San Joaquin light distillate of about 73 SUS at 100° F.

These data clearly demonstrate the remarkable improvement in oxidation stability occasioned by the addition of a maleic anhydride, vinyl acetate, alkyl fumarate polymeric additive to mineral hydrocarbon solvent oils. Thus, the addition of only 6 wt. percent of the polymeric additive significantly reduced the amount of oxidation precipitate formed from the solvent oil indicating that the solvent oil with the additive had superior oxidation stability and would contribute to increased intake system and carburetor cleanliness when incorporated in motor fuels.

#### EXAMPLE 5

To further confirm the superior results and relationship of the Sligh test and the ability of the improved solvent oil composition to reduce intake manifold deposits, additional tests were performed in a Lauson engine. In these tests, the Lauson engine was operated on an experimental gasoline blend similar to a commercial premium grade motor

gasoline, then with the same gasoline containing 0.5 vol. percent of a mineral solvent oil, and finally using a sample of the same gasoline with the same mineral solvent oil containing a small amount of the polymeric additive. After each test, the manifold was washed first with heptane and then with acetone. The solvent was evaporated from the washing and the heptane insoluble acetone soluble deposits weighed and reported in milligrams of deposits per pound of fuel. The solvent oil and polymeric additive were the same as described in Table I. The gasoline used was an experimental premium grade gasoline.

Table II  
EFFECT OF IMPROVED SOLVENT OIL IN A LAUSON ENGINE MANIFOLD TEST

| Test                                                                        | Acetone soluble manifold deposits mg./lb. of gasoline |
|-----------------------------------------------------------------------------|-------------------------------------------------------|
| Gasoline alone                                                              | 2.0                                                   |
| Gasoline plus 0.5 wt. percent solvent oil Y                                 | 1.1                                                   |
| Gasoline plus 0.5 wt. percent solvent oil Y and 0.015 wt. percent polymer D | 0.8                                                   |

From these data, it is apparent that this improvement in oxidation stability as measured by the Sligh test is further reflected in actual Lauson engine tests. The above tests demonstrate that the improved solvent oil compositions effectively reduce manifold deposits to a very low level, and that the improved solvent oil composition is markedly superior to conventional mineral oils alone.

#### EXAMPLE 6

An untreated paraffinic base distillate of about 79 SUS/100° F. from Venezuelan crude is greatly improved in oxidation stability by the addition of about 4 wt. percent of polymer A.

#### EXAMPLE 7

A gasoline solvent oil of enhanced stability characteristics is achieved by the addition of about 8 wt. percent of polymer C to a white oil obtained by exhaustive refining of a naphthene base distillate oil by H<sub>2</sub>SO<sub>4</sub> treating and having a viscosity of about 100 SUS at 100° F.

#### EXAMPLE 8

An improved solvent oil composition characterized by a relatively low tendency to form intake manifold deposits when added at a concentration level of about 0.5 vol. percent to a premium gasoline having a 50% ASTM distillation point of less than 210° F. and an ASTM gum level of more than 5 mg./100 cc. is obtained by the addition of about 3 wt. percent of polymer D and about 1.0 wt. percent of a monobutoxy poly-1,2-oxy propylene glycol and having a viscosity of about 300 SUS at 100° F.

#### EXAMPLE 9

A highly effective solvent oil composition giving beneficial results when incorporated in small quantities, for example 0.3 vol. percent, in a gasoline having more than 20% by weight of catalytically cracked aromatic components is obtained by the admixing of about 60% by volume of an acid treated paraffinic distillate having a SUS viscosity between 75 and 85 at 100° F. and about 35% by volume of acetylated Oxo bottoms obtained by ketene treating Oxo bottoms derived from the oxonation of a butene-propylene copolymer and about 5% by volume of polymer A.

#### EXAMPLE 10

A superior solvent oil having markedly improved oxidation stability is obtained by adding between 2 to 6 wt. percent of polymer D to a silica gel extracted, deasphalted, solvent extracted bright stock solvent oil having less than 5% aromatic content and a pour point less than +30° F.

## EXAMPLE 11

An aviation gasoline with an initial boiling point of about 105° F., a mid boiling point of 210° F., and a final boiling point of about 315° F. is blended with about 4 cc. of tetraethyl lead per gallon, 1 theory of ethylene dibromide and 0.5 vol. percent of a highly refined acid treated and neutralized naphthenic base distillate having a SUS viscosity of about 100 at 100° F. and about 0.01 wt. percent of an ashless oil soluble polymer B. This fuel when used to operate a Continental aviation engine with direct injection contributes to improved engine intake and injection system cleanliness.

## EXAMPLE 12

A highly aromatic motor gasoline containing 60% by volume of a catalytically hydroformed naphtha, a 425° F. ASTM distillation end point, a Reid vapor pressure of about 9 lbs. per square inch and a clear octane number of about 95 is upgraded in manifold and fuel system cleanliness characteristics by the addition of about 0.75 volume percent of a light solvent dewaxed hydrocarbon mineral paraffinic base solvent oil distillate and about 0.008 wt. percent of polymer D.

In summary, the applicants have discovered an improved solvent oil composition having enhanced stability, and which operates to effectively reduce intake system deposits for a far greater degree than conventional solvent oils.

What is claimed is:

1. An improved motor gasoline characterized by a reduced tendency to form objectionable engine deposits, said gasoline containing solvent oil having viscosity of between 50 and 2000 SUS at 100° F. in a minor amount

sufficient to improve upper cylinder lubrication and a very small amount of a polymeric additive sufficient to impart oxidation stability to said solvent oil and to promote engine cleanliness, which polymer is obtained by copolymerizing from 1 to 6 molar percent of maleic anhydride with from 20 to 50 molar percent of a C<sub>8</sub> to C<sub>20</sub> fatty alcohol ester of an α,β-unsaturated C<sub>4</sub> to C<sub>6</sub> dicarboxylic acid and with from 40 to 80 molar percent of a copolymerizable alkenyl C<sub>2</sub> to C<sub>6</sub> ester of an aliphatic monocarboxylic acid to give a polymer having a molecular weight of from 100,000 to 3,000,000.

2. A composition as defined in claim 1 wherein said solvent oil is a hydrocarbon solvent oil and said minor amount is from 0.05 and 3.0 wt. percent.

3. A composition as defined in claim 1 wherein said very small amount is between 0.005 and 0.5 wt. percent.

4. A composition as defined in claim 1 wherein said polymer is obtained by copolymerizing from 1 to 5 molar percent of maleic anhydride with from 20 to 30 molar percent of a C<sub>8</sub> to C<sub>20</sub> fatty alcohol ester of a butenedioic acid and from 65 to 80 molar percent of a vinyl ester of a short chain C<sub>2</sub> to C<sub>4</sub> fatty acid.

## References Cited by the Examiner

## UNITED STATES PATENTS

|           |         |              |       |       |
|-----------|---------|--------------|-------|-------|
| 2,892,690 | 6/1959  | Lowe et al.  | ----- | 44—62 |
| 2,914,479 | 11/1959 | Tom et al.   | ----- | 44—58 |
| 2,927,013 | 3/1960  | Lowe et al.  | ----- | 44—62 |
| 2,995,928 | 10/1960 | Smith et al. | ----- | 44—56 |

## FOREIGN PATENTS

|         |        |                |
|---------|--------|----------------|
| 808,737 | 1/1959 | Great Britain. |
|---------|--------|----------------|

DANIEL E. WYMAN, Primary Examiner.